# EUROPEAN PATENT SPECIFICATION

(11) **EP 1 725 642 B1**
(45) Date of publication and mention of the grant of the patent: **14.05.2008**
(21) Application number: 05725549.9
(22) Date of filing: 15.03.2005
(51) Int. Cl.: C11D 3/37

(54) **SURFACE-TREATING COMPOSITIONS CONTAINING SULFONATED/CARBOXYLATED POLYMERS**
OBERFLÄCHENBEHANDLUNGSMITTEL MIT SULFIERTEN/CARBOXYLIERTEN POLYMEREN
COMPOSITIONS DE TRAITEMENT DE SURFACE CONTENANT DES POLYMERES SULFONES/CARBOXYLES

(30) Priority: 15.03.2004 US 553210 P
(43) Date of publication of application: 29.11.2006
(73) Proprietor: The Procter and Gamble Company, Cincinnati, Ohio 45202 (US); National Starch (Alco Chemical), Chattanooga TN 37406 (US)
(72) Inventor: WAITS, Leslie, Dawn, Cincinnati, Ohio 45220 (US); PRICE, Kenneth, Nathan, Cincinnati, Ohio 45215 (US); DIRR, Penny, Sue, Fairborn, Ohio 45234 (US); SCHNEIDERMAN, Eva, Mason, Ohio 45040 (US); HUTTON, Howard, David, Oregonia, Ohio 45054 (US); SHERRY, Alan, Edward, Cincinnati, Ohio 45220 (US); VINSON, Phillip, Kyle, Fairfield, Ohio 45054 (US); RODRIGUES, Klein, Aloysius, Chattanooga, Tennessee 37377 (US)
(74) Representative: Peet, Jillian Wendy
(86) International application number: PCT/US2005/008459
(87) International publication number: WO 2005/090540

(56) References cited:
- EP-A- 0 798 320
- EP-A- 0 851 022
- WO-A-02/20708
- WO-A-03/060054
- DE-A1- 10 109 799
- DE-A1- 10 233 834
- US-A- 5 547 612
- US-B1- 6 191 088

## Description

### TECHNICAL FIELD

This invention is in the field of cleaning and/or rinsing compositions. More particularly, the invention relates to surface-treating compositions, methods, and compositions of matter, and articles of manufacture containing a water-soluble, sulfonated/carboxylated polymer.

### BACKGROUND OF THE INVENTION

In certain surface-treating compositions and methods, polymers may serve many useful functions. They can function, either independently or concurrently, as thickeners in liquid detergents, as viscosity reducers in the processing of granular detergents, as antiredeposition agents, as scale and deposit inhibitors, as crystal modifiers, and as detergent assistants which are capable of completely or partially replacing the materials used as builders, while imparting to surfactants optimum properties with respect to detergent actions.

In certain applications, use of polycarboxylate polymers may help to reduce hard water filming on substrate surfaces. These polycarboxylate polymers may be derived from (meth)acrylic acids and salts, as well as, from mixtures of such polymers with other compounds and/or polymers, such as phosphonic acids. Copolymers of (meth)acrylic acids and vinyl esters (such as, methyl methacrylate (MMA), ethyl acrylate (EA), hydroxy ethyl methacrylate and hydroxy propyl acrylate), copolymers of (meth)acrylic acids and salts with acrylamido alkyl, aryl sulfonates, or unsubstituted acrylamides, and terpolymers, formed from acrylic acid, 2-acrylamido-2-methyl propane sulfonic acid (AMPS) or unsubstituted acrylamide, are also useful in automatic dishwashing compositions. Polymers comprising polycarboxylates are described in U.S. Pat Nos. 4,745,154; 5,547,612; and 5,591,703.

Recently, several hydrophobic polymers have been developed and are described in U.S. Pat. Nos. 5,489, 397; 5,021,525; 5,534,198; 5,698,312; 5,798,324; 6,395,185; 6,114,294; 4,711,725; and 6,395,185. Sulfonated/carboxylated polymers may exhibit greater levels of hydrophobicity than that seen in conventional polycarboxylates polymers, however, these polymers may be expensive to manufacture, and especially with a high degree of sulfonation (e.g. 4 mole % and greater).

Art related to sulfonated/carboxylated polymers includes: DE 102 3 834 A1; US 6,191,088 B1; US 5,547,612; EP 798,320 A2; EP 851,022 A2; DE 101 09 799 A1; WO 02/20708 and WO 03/060054.

DE 102 3 834 A1 discloses a dishwashing composition comprising a polymer having: i) 30 to 95 mole % of acrylic and/or methacrylic acid or salts thereof; ii) 3 to 35 mole % of a sulfonic acid of certain formula; and iii) 2 to 35 mole % of noniocic monomer of certain formula.

US 6,191,088 B1 discloses an automatic dishwashing composition comprising a water soluble polymer containing sulfonic acid groups which comprises the polymerization product of at least 2.5 mole percent of an allyloxybenzenesulfonic acid monomer of certain structure; at least 0.5 mole percent of methallylsulfonic acid monomer of certain structure; from 10 to 20 mole percent of a copolymerizable non-ionic monomer of certain structure; and at least 60 mole percent of a copolymerizable olefinically unsaturated carboxylic acid monomer.

US 5,547,612 discloses the same polymer as '088.

EP 798,320 A2 relates to a copolymer stable against hydrolysis and useful as a macromolecular surfactant. Specifically, the copolymer is a ternary copolymer comprising (a) unit of a polyoxyalkylene alkenyl ether; (b) unit of alkenylsulfonic acid; and (c) unit of a maleic acid compound. The amount of monomers (a), (b) and (c) fulfils a specific relationship.

EP 851,022 A2 diseases a rinse aid composition containing a polymer having: i) from about 50 wt% to about 99% by weight of an olefinically unsaturated carboxylic acid monomer; and ii) from about 1 wt% to about 50 wt% of at least one monomer unit selected from the group consisting of copolymerizable sulfonated monomers, copolymerizable non-ionic monomers and mixtures thereof.

With regard to the use of some nonionic, amide- and ester-containing monomer in certain automatic dishwashing compositions, this can be actually very problematic. For example, some MMA-containing or AMPS-containing sulfonated/carboxylated polymers are unstable in chlorinated liquid automatic dishwashing compositions (especially in gels having a high pH)-often losing their performance after a couple of weeks in solution. While not wishing to be bound by theory, it is believed that in certain automatic washing detergents these polymers may be subject to attack by chlorine bleach because of the presence of the nitrogen in the amido functionality (such as, in AMPS) or the hydrolysis of the ester linkage (such as, in MMA).

Thus, there remains a long-standing need for surface-treating compositions that comprise more cost-effective polymers. The sulfonated/carboxylated polymers described herein can be used to clean and/or rinse a variety of hard surfaces with good cleaning performance while having less filming, spotting, and/or streaking. For example, these polymers can be used in automatic dishwashing rinse aid compositions, including but not limited to acidic formulations, to help to reduce hard water filming and spotting on tableware surfaces. In some liquid hard surface cleaners (such as, medium-duty detergent compositions or light-duty liquid dishwashing detergents), these polymers can act as an effective hydrotrope to reduce filming and streaking on all types of bathroom and kitchen surfaces, such as tableware, countertops, appliances, fixtures, floors, walls, windows, mirrors, shower doors, etc. These polymers may also be used in other acidic formulations, for example, to clean and/or rinse car surfaces.

Since the sulfonated/carboxylated polymers described herein may contain low sulfonate functionality, they can be more cost-eftectivc than conventional sulfonated/carboxylated polymers with higher sulfonation. When used in a variety of consumer products, these cost-effective polymers provide many consumer benefits. For example, these polymers can be used as processing aids during blending, drying and agglomerating operations, thereby providing uniform distribution of the detergent composition's components, desired particle size and density, as well as, other desirable attributes during manufacture and storage of detergents, especially in powdered detergents (such as, detergent tablets, granulated compact detergents, granulated

automatic dishwashing detergents, and heavy-duty granulated or granular laundry detergents).

Since sulfonated/carboxylated polymers with low sulfonation also provide improved stability performance in the presence of chlorine bleach, they are ideally suited for certain chlorinated and/or highly alkaline detergent compositions (such as liquid or granular, dishwashing detergents and heavy-duty laundry detergents). In the wash liquor, these polymers are believed to perform as a dispersant, co-builder and anti-soil redeposition agent, for both hard surfaces (e.g. tableware) and soft surfaces (e.g. laundry). These polymers are also believed to improve detergency by acting as a co-builder in reducing soil redeposition and water hardness salt deposition in soft surface cleaning applications, as well as, to function as a dispersant, especially in reduced and/or nil builder laundry formulations.

There also remains a need for sulfonated/carboxylated polymers that are hydrophobically modified, inexpensive and yet provide good anti-spotting and anti-filming performance over a broad pH range. Soluble builders, such as conventional hydrotropes, may be added as coupling agents to liquid detergent compositions to improve performance but the use of conventional hydrotropes may be expensive. Another cost-effective approach involves the use of hydrophobically-modified, sulfonated/carboxylated polymers comprising a nonionic functionality that is aimed at permitting interaction with a structured surfactant, thereby giving a stable, concentrated, low viscosity, built, liquid surface-treating composition. Hydrophobically modified, sulfonated/carboxylated polymers outperform conventional hydrotropes by providing an improved stability over a wide range of pH (e.g. both high and low pH formulations). In fact, these hydrophobically-modified, sulfonated/carboxylated polymers offer more flexibility in formulating effective surface-treating compositions than conventional polymers since they may also comprise any suitable level of sulfonate and/or carboxylic acid functionality.

### SUMMARY OF THE INVENTION

In one aspect of the present invention, a domestic, institutional, industrial, and/or commercial surface-treating composition is provided. The surface-treating compositions described herein may comprise: (a) an effective amount of a water-soluble, sulfonated/carboxylated polymer comprising: (i) at least one carboxylic acid functionality; (ii) optionally, one or more nonionic functionality; and (iii) at least one sulfonate functionality, wherein the sulfonate functionality is less than or equal to 2 mole % of the molar content of the polymer; and (b) balance adjunct ingredients.

### DETAILED DESCRIPTION OF THE INVENTION

### Definitions

The sulfonated/carboxylated polymers described herein may be provided in any suitable form including, but not limited to: copolymers, terpolymers, tetrapolymers, interpolymers, and combinations thereof. As used herein the term "copolymer" defines a polymer formed from two monomers, the term "terpolymer" defines a polymer formed from three monomers, the term "tetrapolymer" defines a polymer formed from four monomers, and the term "interpolymer" defines a polymer formed from at least five monomers.

The term "surface," as used herein, encompasses all suitable domestic, institutional, industrial, and/or commercial surfaces that may be cleaned or rinsed. Suitable surfaces include, but are not limited to: hard surfaces, soft surfaces, and combinations thereof. These surfaces may be natural, synthetic, porous, non-porous, woven, non-woven, and combinations thereof. Suitable surfaces include, but are not limited to: glass, plastic, ceramic, metal, fabric, wood, and combinations thereof. Suitable hard surfaces include, but are not limited to: tableware, countertops, furniture, floors, walls, containers, showers, doors, windows, cars, buildings, etc.

The term "tableware," as used herein, encompasses all surfaces used for storing, cooking, serving, and eating food. These tableware surfaces include, but are not limited to: glassware, plasticware, dishware, non-stick cooking surfaces, utensils, etc. Suitable soft surfaces include, but are not limited to: fabrics, linens, clothes, towels, drapes, upholstery, carpets, etc. The term "laundry" as used herein, encompasses all articles of clothing worn by consumers.

The term "effective amount," as used herein, refers to an amount that is sufficient to improve cleaning and/or rinsing of all types of surfaces under normal conditions, or alternatively an amount that is sufficient to reduce hard water filming, streaking, and/or spotting on hard substrate surfaces, to improve whiteness and/or cleaning or to reduce staining and/or soil redeposition on soft surfaces, to improve dispersion of the surface-treating composition in an aqueous medium, such as in wash and/or rinse water, and/or to provide improved product stability performance, especially in the presence of chlorine bleach and high pH.

The term "cleaning device," as used herein, refers to any type of domestic, institutional, industrial, and/or commercial device that is used for cleaning and/or rinsing any suitable surface, such as those described herein. For example, suitable cleaning devices include, but are not limited to: automatic dishwashing (ADW) machines, automatic washing machines for laundry, automatic car wash machines, sinks, buckets, pressure washers, garden hose attachments, and combinations thereof. The cleaning device may be portable, semi-portable, or fixed (such as, a fixture). For example, a hand-held cleaning device (e.g. spray washer, mop, etc.) could comprise any suitable sulfonated/carboxylated polymer containing-fluid source (e.g. fluid container, water line, water hose, etc.).

### Sulfonated/carboxylated Polymers

This invention is useful for treating surfaces with compositions, methods, compositions of matter, and articles of manufacture comprising a surface-treating composition. The surface-treating compositions described herein may comprise any suitable sulfonated/carboxylated polymer described herein in any suitable amount. In one non-limiting embodiment, the surface-treating composition may comprise from about 0.01% to about 100%, or from about 0.01% to about 99%, or from about 0.01% to about 95%, or from about 0.01 % to about 90%, or from about 0.01% to about 80%, or from about 0.01 % to about 70%, or from about 0.01 % to about 60%, or from about 0.01 % to about 50%, or from about 0.01 % to about 40%, or from about 0.01 % to about 30%, or from about 0.01% to about 20%, or from about 0.0 1 % to about 10%, or from about 0.01% to about 5%, or from about 0.01% to about 4%, or from about 0.01% to about 3%, or from about 0.01% to about 2%, or alternatively from about 0.01% to about 1%, by weight of the composition, of a suitable sulfonated/carboxylated polymer described herein.

Suitable sulfonated/carboxylated polymers described herein may have a weight average molecular weight of less than or equal to about 100,000 Da, or less than or equal to about 75,000 Da, or less than or equal to about 50,000 Da, or from about 10,000 Da to about 50,000, or from about 15,000 Da to about 50,000 Da; or from about 20,000 Da to about 50,000 Da, or alternatively from about 25,000 Da to about 50,000 Da.

As noted herein, the sulfonated/carboxylated polymers may comprise (a) at least one structural unit derived from at least one carboxylic monomer having the general formula (I): wherein R¹ to R⁴ are independently hydrogen, methyl, carboxylic acid group or CH₂COOH and wherein the carboxylic acid groups can be neutralized; (b) optionally, one or more structural units derived from at least one nonionic monomer having the general formula (II): wherein R⁵ is hydrogen, C₁ to C₆ alkyl, or C₁ to C₆ hydroxyalkyl, and X is either aromatic (with R⁵ being hydrogen or methyl when X is aromatic) or X is of the general formula (III): wherein R⁶ is (independently of R⁵) hydrogen, C₁ to C₆ alkyl, or C₁ to C₆ hydroxyalhyl, and Y is O or N; and at least one structural unit derived from at least one sulfonate monomer having the general formula (IV): wherein R⁷ is a group comprising at least one sp² bond, A is O, N, P, S or an amido or ester linkage, B is a mono- or polycyclic aromatic group or an aliphatic group, each t is independently 0 or 1, and M⁺ is a cation. In one aspect, R⁷ is a C₂ to C₆ alkene. In another aspect, R⁷ is ethane, butene or propene.

### Sulfonated/carboxylated Polymer with Low Sulfonate Functionality (SMPLSF)

The surface-treating compositions of the present invention may incorporate a cost-effective, water-soluble, sulfonated/carboxylated polymer with low sulfonate functionality, which is hereinafter referred to therein as an "SMPLSF."

The at least one carboxylic acid functionality of a suitable SMPLSF may be present in any suitable amount. For example, the at least one carboxylic acid functionality may be present in any suitable amount less than or equal to about 0.01 mole %, or less than or equal to about 0.1 mole % or less than or equal to about 1 mole %, or less than or equal to about 2 mole %, or less than or equal to about 5 mole %, or less than or equal to about 10. mole %, or less than or equal to about 20 mole %, or less than or equal to about 30 mole %, or less than or equal to about 40 mole %, or less than or equal to about 50 mole %, or less than or equal to about 55 mole %, or less than or equal to about 60 mole %, or less than or equal to about 65 mole %, or less than or equal to about 70 mole %, or less than or equal to about 75 mole %, or less than or equal to about 80 mole %, or less than or equal to about 85 mole %, or less than or equal to about 90 mole %, or less than or equal to about 95 mole %, or alternatively less than or equal to about 99.99 mole % of the total SMPLSF molar content.

The optional one or more nonionic functionality of a suitable SMPLSF may be present, if at all, in any suitable amount to provide hydrophobicity. For example, when present, the one or more nonionic functionality may be greater than or equal to about 0.01 mole %, or greater than or equal to about 0.1 mole %, or greater than or equal to about 1 mole %, or greater than or equal to about 2 mole %, or greater than or equal to about 3 mole %, or greater than or equal to about 4 mole %, or greater than or equal to about 5 mole %, or greater than or equal to about 10 mole %, or greater than or equal to about 20 mole %, or greater than or equal to about 30 mole %, or greater than or equal to about 40 mole %, or greater than or equal to about 50 mole %, or greater than or equal to about 60 mole %, or greater than or equal to about 70 mole %, or greater than or equal to about 80 mole %, or greater than or equal to about 90 mole %, or greater than or equal to about 95 mole %, or alternatively greater than or equal to about 99.98 mole % of the total SMPLSF molar content.

The at least one sulfonate functionality of a suitable SMPLSF may be present in any suitable amount less than or equal to 2 mole %. For example, the sulfonate functionality may be present at a level less than or equal to 1.5 mole %, or less than or equal to about 1 mole %, or less than or equal to about 0.5 mole %, or equal to about 0.1 mole %, or alternatively less than or equal to about 0.01 mole % of the total SMPLSF molar content.

In one non-limiting embodiment, a suitable SMPLSF may comprise: (a) from 0.01 mole % to 2 mole % of at least one sulfonate functionality; and (b) less than or equal to 99.99 mole % of a carboxylic acid functionality. In another non-limiting embodiment, this SMPLSF may be free of an ester and/or an amide functionality.

In another non-limiting embodiment, a suitable SMPLSF may comprise: (a) from 0.01 mole % to 50 mole % of at least one nonionic functionality; (b) from 0.01 mole % to less than or equal to 2 mole % of at least one sulfonate functionality; and (c) from 99.98 mole % to 48 mole % of a acid functionality. In another non-limiting embodiment, this SMPLSF may comprise an aromatic monomer, such as styrene.

In another non-limiting embodiment, the at least one carboxylic acid functionality can comprise one or more of the following: acrylic acid, maleic acid, itaconic acid, methacrylic acid, or ethoxylate esters of acrylic acids. In another non-limiting embodiment, the sulfonate functionality can comprise one or more of the following: sodium (meth) allyl sulfonate, vinylsulfonate, sodium phenyl (meth) allyl ether sulfonate, or 2-acrylamido-methyl propane sulfonic acid. In another non-limiting embodiment, the optional one or more nonionic functionality can comprise one or more of the following: methyl (meth) acrylate, ethyl (meth) acrylate, t-butyl (meth) acrylate, methyl (meth) acrylamide, ethyl (meth) acrylamide, t-butyl (meth) acrylamide, styrene, or α-methyl styrene. In another non-limiting embodiment, a surface-treating composition may comprise an SMPLSF comprising styrene, having a molecular weight of less than or equal to about 100,000 Da.

### Stability

In one non-limiting embodiment, the SMPLSF may be chemically stable is the surface-treating composition described herein in the presence of bleach and/or high pH. It is believed that stability of the SMPLSF is improved when an effective amount of one or more nonionic functionality is present, especially when the SMPLSF is free of an ester and/or amide functionality. This is not only useful for chlorine-containing and/or highly alkaline detergent products, but also in a chlorine- containing and/or highly alkaline wash water of a cleaning device (e.g. an automatic washing machine or dishwashing machine) where an ester and/or an amide functionality can be hydrolyzed and attacked in solution.

### Hydrophobically Modified Polymer (HMP)

The surface-treating compositions of the present invention may also exhibit enhanced hard water anti-filming performance and improved product stability at a cheaper cost by incorporating a water-soluble, hydrophobically modified polymer comprising an effective amount of one or more nonionic monomers, at least one sulfonate-containing monomer, and at least one carboxylic acid-containing monomer, which is hereinafter referred to as an "HMP."

The one or more nonionic functionality may be greater than or equal to about 0.01 mole %, or greater than or equal to about 0.1 mole %, or greater than or equal to about 1 mole %, or greater than or equal to about 2 mole %, or greater than or equal to about 3 mole %, or greater than or equal to about 4 mole %, or greater than or equal to about 5 mole %, or greater than or equal to about 10 mole %, or greater than or equal to about 20 mole %, or greater than or equal to about 30 mole %, or greater than or equal to about 40 mole %, or greater than or equal to about 50 mole %, or greater than or equal to about 60 mole %, or greater than or equal to about 70 mole %, or greater than or equal to about 80 mole %, or greater than or equal to about 90 mole %, or greater than or equal to about 95 mole %, or alternatively greater than or equal to about 99.98 mole % of the total HMP molar content.

The at least one carboxylic acid functionality and/or at least one sulfonate functionality of a suitable HMP may be present in any suitable amount. For example, any of these functionalities may be present in any suitable amount less than or equal to about 0.01 mole %, or less than or equal to about 0.02 mole %, or less than or equal to about 0.1 mole %, or less than or equal to about 1 mole %, or less than or equal to about 2 mole %, or less than or equal to about 5 mole %, or less than or equal to about 10 mole %, or less than or equal to about 20 mole %, or less than or equal to about 30 mole %, or less than or equal to about 40 mole %, or less than or equal to about 50 mole %, or less than or equal to about 55 mole %, or less than or equal to about 60 mole %, or less than or equal to about 65 mole %, or less than or equal to about 70 mole %, or less than or equal to about 75 mole %, or less than or equal to about 80 mole %, or less than or equal to about 85 mole %, or less than or equal to about 90 mole %, or less than or equal to about 95 mole %, or alternatively less than or equal to about 99.98 mole % of the total HMP molar content.

The at least one nonionic functionality may be selected from the group consisting of methyl (meth) acrylate, ethyl (meth) acrylate, t-butyl (meth) acrylate, methyl (meth) acrylamide, ethyl (meth) acrylamide, t-butyl (meth) acrylamide, styrene, α-methyl styrene, and combinations thereof In another non-limiting embodiment, the HMP may comprise one or more nonionic monomers that may be free of an ester and/or an amide functionality. A suitable example of one or more nonionic monomers that do not contain an ester and/or amide functionality includes, but is not limited to, an aromatic monomer (such as, styrene).

### pH

Any suitable pH may be used herein. A suitable pH may be from about 1 to about 14, when measured at a 1% concentration in an aqueous solution unless otherwise noted. In certain non-limiting embodiments, the surface-treating composition may exhibit an alkaline pH in the range of from about 8 to about 14, or from about 9 to about 12.5, from about 9 to about 11.5, or alternatively from about 9 to about 10. These alkaline surface-treating compositions may comprise chlorine, bleach. In certain other none-limiting embodiments, the surface-treating composition may exhibit an acidic pH in the range of from about 1 to about 6.5, or from about 1 to about 6, or from about 1 to about 5, or from about 1 to about 4, or from about 1 to about 3 or alternatively from about 1 to about 2.

In the case of automatic washing detergent compositions (such as, dishwashing detergents and heavy-duty or laundry detergents), mildly- to highly-alkaline compositions may be effectively used. However, in the case of hard surface cleaners (such as, medium-duty detergents and light-duty liquid detergents) less alkaline compositions may be desirable, especially when mildness to skin is a concern. In certain rinse aid compositions, a lower pH range may tend to reduce incompatibility and negative interaction with existing commercial product residues left in the dispenser reservoir of the automatic dishwashing machine prior to use.

### ADJUNCT INGREDIENTS

Any suitable adjunct ingredient in any suitable amount may be used in the surface-treating compositions described herein. Suitable adjunct ingredients include, but are not limited to: aesthetic agents, anti-filming agents, antiredopsition agents, anti-spotting agents, beads, binders, bleach activators, bleach catalysts, bleach stabilizing systems, bleaching agents, brighteners, buffering agents, builders, carriers, chelants, clay, color speckles, control release agents, corrosion inhibitors, dishcare agents, disinfectant, dispersant agents, dispersant polymers, draining promoting agents, drying agents, dyes, dye transfer inhibiting agents, enzymes, enzyme stabilizing systems, fillers, free radical inhibitors, fungicides, germicides, hydrotropes, opacifiers, perfumes, pH adjusting agents, pigments, processing aids, silicates, soil release agents, suds suppressors, surfactants, stabilizers, thickeners, zeolite, and mixtures thereof.

Suitable builders include, but are not limited to: alkali metals; ammonium and alkanolammonium salts of polyphosphates, alkali metal silicates, alkaline earth and alkali metal carbonates, nitrilotriacetic acids, polycarboxylates, (such as, citric acid, mellitic acid, succinic acid, oxydisuccinic acid, polymaleic acid, benzene 1,3,5-tricarboxylic acid, carboxymethyloxysuccinic acid, the water-soluble salts thereof), phosphates (e.g. sodium tripolyphosphate), and mixtures thereof. Suitable enzymes include, but are not limited to: proteases, amylases, cellulases, lipases, carbohydrases, bleaching enzymes, cutinases, esterases, and wild-type enzymes. Suitable surfactants include, but are not limited to: nonionic surfactants, anionic surfactants, cationic surfactants, ampholytic surfactants, zwitterionic surfactants, and mixtures thereof. Suitable bleaching agents include, but are not limited to: common inorganic/organic chlorine bleach (such as, sodium or potassium dichloroisocyanurate dihydrate, sodium hypochlorite, sodium hypochloride), hydrogenperoxide releasing salt (such as, sodium perborate monohydrate (PB1), sodium perborate tetrahydrate (PB4)), sodium percarbonate, sodium peroxide, and mixtures thereof. Suitable bleach-modifying materials, include but are not limited to: hydrogen peroxide-source bleach activators (e.g. TAED), bleach catalysts (e.g. transition containing cobalt and manganese). Suitable carriers include, but are not limited to: water, low molecular weight organic solvents (such as, primary alcohols, secondary alcohols, monohyric alcohols, polyols, and mixtures thereof), and mixtures thereof.

Suitable acids include, but are not limited to: acetic acid, aspartic acid, benzoic acid, boric acid, bromic acid, citric acid, formic acid, gluconic acid, glutamic acid, hydrochloric acid, lactic acid, malic acid, nitric acid, sulfamic acid, sulfuric acid, tartaric acid, and mixtures thereof. Suitable corrosion inhibitors, include, but are not limited to: soluble metal salts, insoluble metal salts, and mixtures thereof. Suitable metal salts include, but are not limited to: aluminum, zinc (e.g. hydrozincite), magnesium, calcium, lanthanum, tin, gallium, strontium, titanium, and mixtures thereof). Suitable aesthetic agents include, but are not limited to: opacifiers, dyes, pigments, color speckles, beads, brighteners, and mixtures thereof.

In one non-limiting embodiment, the surface-treating composition may comprise a liquid, gel, or liquigel having a viscosity of from 50 cps to 2000 cps, or alternatively from 100 cps to 350 cps, measured with a Brookfield Viscometer, with a No. 1.8 spindle, at 20° C. These surface-treating compositions can also comprise any suitable solvent in any suitable amount (such as, an effective amount so as to reach the desired viscosity).

With the addition of suitable adjuncts, the surface-treating compositions described herein could be useful as automatic dishwashing detergent (ADD) compositions (e.g. builders, surfactants, enzymes, etc.), light-duty liquid dishwashing compositions, laundry compositions such as, compact and heavy-duty detergents (e.g. builders, surfactants, enzymes, etc.), rinse aid compositions (e.g. acid, nonionic low-foaming surfactants, carrier, etc.), and/or hard surface cleaning compositions (e.g. zwitterionic surfactants, germicide, etc.).

Suitable adjunct ingredients are disclosed in one or more of the following: U.S. Pat. Nos. 2,798,053; 2,954,347; 2,954,347; 3,308,067; 3,314,891; 3,455,839; 3,629,121; 3,723,322; 3,803,285; 3,929,107; 3,929,678; 3,933,672; 4,133,779; 4,141,841; 4,228,042; 4,239,660; 4,260,529; 4,265,779; 4,374,035; 4,379,080; 4,412,934; 4,483,779; 4,483,780; 4,536,314; 4,539,130; 4,565,647; 4,597,898; 4,606,838; 4,634,551; 4,652,392; 4,671,891; 4,681,592; 4,681,695; 4,681,704; 4,686,063; 4,702,857; 4,968,451; 5,332,528; 5,415,807; 5,435,935; 5,478,503; 5,500,154; 5,565,145; 5,670,475; 5,942,485; 5,952,278; 5,990,065; 6,004,922 ;6,008,181; 6,020,303; 6,022,844; 6,069,122; 6,060,299; 6,060,443; 6,093,856; 6,130,194; 6,136,769; 6,143,707; 6,150,322; 6,153,577; 6,194,362; 6,221,825; 6,365,561; 6,372,708; 6,482,994; 6,528,477; 6,573,234; 6,589,926; 6,627,590; 6,645,925; and 6,656,900; WO Pat. Nos. 00/23548; 00/23549; 00/47708; 01/32816; 01/42408; 91/06637; 92/06162; 93/19038; 93/19146; 94/09099; 95/10591; 95/26393; 98/35002; 98/35003; 98/35004; 98/35005; 98/35006; 99/02663; 99/05082; 99/05084; 99/05241; 99/05242; 99/05243; 99/05244; 99/07656; 99/20726; and 99/27083; EP Pat. No. 130756; GB-A-1137741; Chemtech, March 1993, pp 30-33, and J. American Chemical Soc., 115, 10083-10090 (1993); and Kirk Othmer Encyclopedia of Chemical Technology, Third Edition, Volume 7, pages 430-447 (John Wiley & Sons, Inc., 1979).

In one non-limiting embodiment, the surface-treating composition may comprise from 0% to about 99.99%, or from about 0.01% to about 95%, or from about 0.01 % to about 90%, or from about 0.01% to about 80%, or from about 0.01% to about 70%, or from about 0.01% to about 60%, or from about 0.01% to about 50%, or from about 0.01% to about 40%, or from about 0.01% to about 30%, or from about 0.01% to about 20%, or from about 0.01% to about 10%, or from about 0.01% to about 5%, or from about 0.01% to about 4%, or from about 0.01% to about 3%, or from about 0.01% to about 2%, or from about 0.01 % to about 1 %, or from about 0.01 % to about 0.5%, or alternatively from about 0.01% to about 0.1%, by weight of the composition, of a suitable adjunct ingredient.

### PRODUCT FORM

The surface-treating composition can be provided in any suitable physical form. A suitable form may include, but is not limited to: solids; granules; powder; liquid; paste; cream; gel; liquigels, and combinations thereof. The surface-treating compositions used herein can comprise a unitized dose in one of the following forms: tablets, multi-phase tablets, gel pacs, capsules, multi-compartment capsules, water-soluble pouches, or multi-compartment pouches. The surface-treating composition can be dispensed from any suitable device. Suitable devices include, but are not limited to: wipes, hand mittens, boxes, baskets, bottles (e.g. pourable bottles, pump assisted bottles, squeeze bottles), multi-compartment bottles, jars, paste dispensers, and combinations thereof.

In the case of additive or multi-component products contained in single- and/or multi-compartment pouches, capsules, or bottles, it is not required that the adjunct ingredients nor the surface-treating compositions be in the same physical form. In one non-limiting embodiment, the surface-treating composition can provide in a multi-compartment, water-soluble pouch comprising both a solid and a liquid or gel component in a unit dose form. The presence of different forms may allow for a controlled release (e.g. delayed, sustained, triggered or slow release) of the surface-treating composition during treatment of a surface (e.g. during one or more wash and/or rinse cycles in an automatic dishwashing machine).

### Water-soluble Pouch

Many of the surface-treating compositions described herein may demonstrate improved compatibility with partially hydrolysed, water-soluble polyvinyl alcohol (PVA) pouch materials of known construction and type. This is particularly surprising given that many well-known polar/or hydrolysed bonding solvent materials (for example the organoamines) in themselves have low compatibility with PVA materials and present serious issues for product stability.

### METHOD OF USE / COMPOSITION OF MATTER

Any suitable domestic, institutional, industrial, and/or commercial method of treating a surface may be used in herein. In the methods described herein, any suitable surface-treating composition may be used, alone or in combination with a composition of matter (such as the wash and/or rinse water), and/or as part of an article of manufacture comprising a kit having a composition comprising an effective amount of a suitable sulfonated/carboxylated polymer. Any suitable surface may be treated with the sulfonated/carboxylated polymer described herein.

In one non-limiting embodiment, the method may comprise the step of contacting a surface with a surface-treating composition comprising the sulfonated/carboxylated polymer described herein. In another non-limiting embodiment, the method may comprise the step of contacting tableware, especially glass and plastic, in a cleaning device (e.g. an automatic dishwashing machine) with a composition of matter comprising a wash and/or rinse water having a concentration from about 1 ppm to about 10,000 ppm by concentration, of the above described surface-treating composition, as delivered to the tableware surface via the cleaning device. In other non-limiting embodiments, the method may comprise the step of contacting laundry with a composition of matter comprising a wash and/or rinse water having a concentration from about 1 ppm to about 10,000 ppm by concentration, of the above-described surface-treating composition, as delivered to the laundry surface via a cleaning device (e.g. an automatic washing machine). In other non-limiting embodiments, the method may comprise the step of contacting a car surface with a composition of matter comprising a wash and/or rinse water having a concentration from about 1 ppm to about 10,000 ppm by concentration, of the above-described surface-treating composition, as delivered to the car surface via a cleaning device (e.g. an automatic car wash or hand-held pressure washer).

### EXAMPLES

### EXAMPLE 1

A surface-treating composition of the present invention may incorporate any suitable sulfonated/carboxylated polymer described herein. To prepare a suitable sulfonated/carboxylated polymer comprising acrylic acid ('AA'), styrene, sodium methallylsulfonate ('SMS') and sodium phenylmethallylether ('SPME') in the mole ratio 89:10:0.57:0.43, an initial charge of 150 g deionized water, 120 g isopropyl alcohol, 3.2 grams SMS and 4.0 grams SPME was added to a 1-liter glass reactor fitted with a lid and having inlet ports for an agitator, water cooled condenser and for the addition of monomer and initiator solutions. The reactor contents were heated to reflux (approximately 85°C). At reflux, continuous additions of 226 g of acrylic acid and 36.1 g of styrene were added concurrently to the reactor with stirring over a period of 3 hours. During the same time period and for 30 additional minutes, an initiator solution of 13.3 grams sodium persulfate dissolved in 80 grams water was also added. At the end of the initiator addition, a 50% aqueous sodium hydroxide solution (251 g) along with 100 grams water was added. The alcohol co-solvent (approximately 200 grams) was removed from the polymer solution by azeotropic distillation.

The surface-treating compositions described herein can be suitably prepared and packaged by any process chosen by the formulator, non-limiting examples of which are described in U.S. Pat. Nos. 4,005,024 issued Jan. 25, 1977; 4,237,155 issued Dec. 2, 1980; 5,378,409 issued Jan. 3, 1995; 5,486,303 issued Jan. 23, 1996; 5,489,392 issued Feb. 6, 1996; 5,516,448 issued May 14, 1996; 5,565,422 issued Oct. 15, 1996; 5,569,645 issued Oct. 29, 1996; 5,574,005 issued Nov. 12, 1996; 5,599,400 issued Feb. 4, 1997; 5,599,786 issued Feb. 4, 1997; 5,691,297 issued Nov. 11, 1997; 5,698,505 issued Dec. 16, 1997; 5,703,034 issued Dec. 30, 1997; 5,768,918 issued Jun. 23, 1998; 5,891,836 issued Apr. 6, 1999; 5,952,278 issued Sep. 14, 1999; 5,952,278 issued Sep. 14, 1999; 5,968,539 issued Oct. 19, 1999; 5,990,065 issued Nov. 23, 1999; 6,069,122 issued May 30, 2000; 6,147,037 issued Nov. 14, 2000; 6,156,710 issued Dec. 5, 2000; 6,162,778 issued Dec. 19, 2000; 6,180,583 issued Jan. 30, 2001; 6,183,757 issued Feb. 6, 2001; 6,190,675 issued Feb. 20, 2001; 6,204,234 issued Mar. 20, 2001; 6,214,363 issued Apr. 10, 2001; 6,251,845 issued Jun. 26, 2001; 6,274,539 issued Aug. 14, 2001; 6,281,181 issued Aug. 28, 2001; 6,365,561 issued Apr. 2, 2002; 6,372,708 issued Apr. 16, 2002; 6,444,629 issued Sep. 3, 2002; 6,451,333 issued Sep. 17, 2002; 6,482,994 issued Nov. 19, 2002; 6,528,477 issued Mar. 4, 2003; 6,559,116 issued May 6, 2003; 6,573,234 issued Jun 3, 2003; 6,589,926 issued Jul. 8, 2003; 6,627,590 issued Sep. 30, 2003; 6,627,590 issued Sep. 30, 2003; 6,630,440 issued Oct. 7, 2003; 6,645,925 issued Nov. 11, 2003; and 6,656,900 issued .Dec. 2, 2003; U.S. Pat. Appl. Nos. 20030228998 to Dupont published Dec. 2003; US20010026792 to Farrell et al. published Oct. 2001; 20010031714 to Gassenmeier et al.published Oct. 2001; 20020004472 to Holderbaum et al. published Jan. 2002; 20020004473 to Busch et al. published Jan. 2002; 20020013232 to Kinoshita et al. published Jan. 2002; 20020013242 to Baillely et al. published Jan. 2002; 20020013243 to Brown published Mar. 2002; 20020028756 to Carter et al. published Mar. 2002; 20020033004 to Edwards et al. published Mar. 2002; 20020045559 to Forth et al. published Apr. 2002; 20020055449 to Porta et al. published May 2002; 20020094942 to Danneels et al. published July 2002; 20020119903 to Lant et al. published Aug. 2002; 20020123443 to Bennie et al. published Sep. 2002; 20020123444 to Fisher et al. published Sep. 2002; 20020137648 to Sharma et al. published Sep. 2002; 20020166779 to Etesse et al. published Nov. 2002; 20020169092 to Catlin et al. published Nov. 2002; 20020169095 to Forth et al. Nov. 2002; and 20020198125 to Jones published Dec 2002.

Tables I-III provide non-limiting product formulations of suitable ADD compositions. Table IV provides non-limiting product formulations of suitable rinse aid compositions. Tables V and VI provide non-limiting product formulations of suitable laundry detergents. Table VII provides non-limiting product formulations of suitable hard surface cleaning compositions. Table VIII provides non-limiting product formulations of suitable light-duty liquid detergent compositions. Tables IX and X provide the chemical composition and name of some non-limiting examples of sulfonated/carboxylated polymers described herein.

**TABLE I**

| Liquid/Gel ADD Composition | | | | | | |
|---|---|---|---|---|---|---|
| INGREDIENTS | EXAMPLES | | | | | |
| | 2 | 3 | 4 | 5 | 6 | 7 |
| STPP / SKTP / KTPP | 17.5 | 17.5 | 17.5 | 17.5 | 22.0 | 22.0 |
| Polymer¹ | 0.5 | 1.0 | 2.0 | 4.0 | 0.5 | 2.0 |
| Sodium hydroxide | 1.9 | 1.9 | 1.9 | 1.9 | - | - |
| Potassium hydroxide | 3.9 | 3.9 | 3.9 | 3.9 | 5.8 | 5.8 |
| Sodium silicate | 7.0 | 7.0 | 7.0 | 7.0 | - | - |
| H2SO4 | - | - | - | - | 3.9 | 3.9 |
| Thickener | 1.0 | 1.0 | 1.0 | 1.0 | 1.2 | 1.2 |
| Sodium hypochlorite | 1.2 | 1.2 | 1.2 | 1.2 | - | - |
| Nonionic surfactant | - | - | - | - | 1.0 | 1.0 |
| Protease enzyme | - | - | - | - | 0.6 | 0.6 |
| Amylase enzyme | - | - | - | - | 0.2 | 0.2 |
| Enzyme stabilizing agents | - | - | - | - | 3.5 | 3.5 |
| Water and minors | Balance | Balance | Balance | Balance | Balance | Balance |
| pH (1% Solution) | 11.7 | 11.7 | 11.7 | 11.7 | 9 | 9 |

| | | | | | | |
|---|---|---|---|---|---|---|
| 1 Hydrophobically modified, sulfonated/carboyxlated polymer "E" with 80.9 mole % AA, 0 mole % MA, 18 mole % STY, 0.62% SMS and 0.5 mole % SPME. 2 Balance to 100% can, for example, include dyes, perfumes, speckles, corrosion inhibitor, dishcare agent, fillers, solvents, polymers, and additional water. | | | | | | |

**TABLE II**

| Granular Or Powder ADD Composition | | | | | | | |
|---|---|---|---|---|---|---|---|
| INGREDIENTS | EXAMPLES | | | | | | |
| | 8 | 9 | 10 | 11 | 12 | 13 | 14 |
| STPP / SKTP / KTPP | 20.0 | 20.0 | 23.0 | 23.0 | 23.0 | 28.0 | - |
| Sodium citrate | - | - | - | - | - | - | 25 |
| Hydrozincite | - | 0.05 | 0.10 | 0.15 | 0.5 | 0.1 | 0.1 |
| Polymer¹ | 1.0 | 1.0 | 1.0 | 1.0 | 1.0 | 1.0 | 1.0 |
| Sodium carbonate | 30.0 | 30.0 | 30.0 | 30.0 | 30.0 | 30.0 | 30.0 |
| Sodium silicate | 5.5 | 5.5 | 5.5 | 5.5 | 5.5 | 5.5 | 5.5 |
| Surfactant | 0.9 | 0.9 | 0.9 | 0.9 | 0.9 | 1.8 | 0.9 |
| Polymer Dispersant² | - | - | - | - | - | 3.3 | - |
| Sodium perborate | 4.3 | 4.3 | 4.3 | 4.3 | 4.3 | 4.3 | 4.3 |
| Bleach catalyse | 0.004 | 0.004 | 0.004 | 0.004 | 0.004 | 0.004 | 0.004 |
| Protease enzyme | 0.6 | 0.6 | 0.6 | 0.6 | 0.6 | 1.0 | 0.25 |
| Amylase enzyme | 0.2 | 0.2 | 0.2 | 0.2 | 0.2 | 0.2 | 0.13 |
| Water and minors⁴ | Balance | Balance | Balance | Balance | Balance | Balance | Balance |
| pH (1% Solution) | 10 | 10 | 10 | 10 | 10 | 10 | 10 |

| | | | | | | | |
|---|---|---|---|---|---|---|---|
| 1 Hydrophobically modified, sulfonated/carboyxlated polymer "E" with 80.9 mole % AA, 0 mole % MA, 18 mole % STY, 0.62% SMS and 0.5 mole % SPME. 2 PEI 189 E15-18 according to U.S. Pat. No. 4,597,898 Vander Meer, issued Jul. 1, 1986. 3 5,12-dimethyl-1,5,8,12-tetraaza-bicyclo[6.6.2]hexadecanemanganese (II) chloride. 4 Balance to 100% can, for example, include dyes, perfumes, speckles, corrosion inhibitor, dishcare agent, fillers, solvents, and other polymers. | | | | | | | |

**TABLE III**

| ADD Compositions in Water-Soluble Pouches⁴ | | | | | |
|---|---|---|---|---|---|
| INGREDIENTS | EXAMPLES | | | | |
| | 15 | 16 | 17 | 18 | 19 |
| STPP / SKTP / KTPP | 33.0 | 33.0 | 33.0 | 33.4 | 30.7 |
| Sodium citrate | - | - | - | - | 33.6 |
| Polymer¹ | 1.0 | 1.0 | 1.0 | 1.0 | 1.0 |
| Sodium carbonate | 19.0 | 19.0 | 28.0 | 26.0 | - |
| Sodium silicate | 7.8 | 7.8 | 4.2 | 4.3 | - |
| Surfactant | 3.2 | 3.2 | 6.5 | 2.3 | 0.5 |
| Dispersant polymer | - | - | 4.3 | - | - |
| NaDCC / sodium hypochloride | - | - | - | 1.1 | - |
| Sodium perborate | 12.8 | 12.8 | 9.3 | - | - |
| Bleach catalyst² | 0.013 | 0.013 | 1.4 | - | - |
| Protease enzyme | 2.2 | 2.2 | 0.3 | - | 1.3 |
| Amylase enzyme | 1.7 | 1.7 | 0.9 | - | 0.2 |
| Water and minors³ | Balance | Balance | Balance | Balance | Balance |
| pH (1% Solution) | 10 | 10 | 10 | 10 | 10 |

| | | | | | |
|---|---|---|---|---|---|
| 1 Hydrophobically modified, sulfonated/carboyxlated polymer "E" with 80.9 mole % AA, 0 mole % MA, 18 mole % STY, 0.62% SMS and 0.5 mole % SPME. 2 5,12-dimethyl-1,5,8,12-tetraaza-bicyclo[6.6.2]hexadecanemanganese (II) chloride. 3 Balance to 100% can, for example, include dyes, perfumes, speckles, corrosion inhibitor, dishcare agent, fillers, solvents, polymers, and additional water. 4 Single-compartment or multiple-compartmented water-soluble pouches comprised of partially hydrolyzed, water-soluble polyvinyl alcohol. | | | | | |

**TABLE IV**

| Rinse Aid Composition | | | | | |
|---|---|---|---|---|---|
| INGREDIENTS | EXAMPLES | | | | |
| | 20 | 21 | 22 | 23 | 24 |
| Polymer¹ | 1.0 | 4.0 | 5.0 | 5.0 | 10.0 |
| Nonionic Surfactant | 35.0 | 35.0 | 35.0 | 35.0 | 20.0 |
| Acid | - | 1.2 | 1.56 | - | - |
| Chelating Agent | - | - | - | - | 20.0 |
| Polymer Dispersant² | - | - | 4.0 | - | - |
| Perfume | 0.12 | 0.12 | 0.12 | 0.12 | - |
| Water and minors³ | Balance | Balance | Balance | Balance | Balance |
| pH (1% Solution) | 6.5 | 2.6 | 2.6 | 2.8 | 2.8 |

| | | | | | |
|---|---|---|---|---|---|
| 1 Hydrophobically modified, sulfonated/carboyxlated polymer "E" with 80.9 mole % AA, 0 mole % MA, 18 mole % STY, 0.62% SMS and 0.5 mole % SPME. 2 PEI 189 E15-18 according to U.S. Pat..No. 4,597,898 Vander Meer, issued Jul. 1, 1986. 3 Balance to 100% can, for example, include dyes, perfumes, speckles, corrosion inhibitor, dishcare agent, hydrotropes, solvents, polymers, and additional water. | | | | | |

**TABLE V**

| Granular Heavy-Duty Laundry Detergent Composition | | | | | | | |
|---|---|---|---|---|---|---|---|
| INGREDIENTS | EXAMPLES | | | | | | |
| | 26 | 27 | 28 | 29 | 30 | 31 | 32 |
| Anionic surfactant | 22 | 18 | 20 | 20 | 10.6 | 10.6 | 28 |
| Nonionic surfactant | 1.5 | 0.5 | 1.1 | 1.1 | 9.4 | 9.4 | 3.3 |
| Cationic surfactant | - | - | 0.7 | 0.7 | - | - | 0.5 |
| Zeolite | 28 | 25 | - | - | 24 | 24 | 11 |
| Phosphate | - | - | 25 | 25 | - | - | - |
| Silicate | - | - | - | - | 8.5 | 8.5 | 7.5 |
| Sodium carbonate/ bicarbonate | 27 | 19 | 14 | 14 | 8.9 | 8.9 | 15 |
| Sodium sulfate | 5.4 | 11 | 15 | 15 | 11 | 11 | 3.5 |
| Sodium silicate | 0.6 | 1.1 | 10 | 10 | - | - | 12 |
| Enzymes | 0.4 | 0.4 | 1.6 | 1.6 | 1.5 | 1.5 | 0.2 |
| Polyamine | 4.3 | 6.5 | 1.9 | 1.9 | 5.0 | 5.0 | 0.7 |
| Polymer¹ | 1.0 | 1.0 | 1.0 | - | - | - | - |
| Polymer² | - | - | - | 1.0 | 1.0 | 1.0 | 1.0 |
| Chelants | - | 0.5 | - | 1.0 | 0.5 | 0.5 | - |
| Brighteners | 0.2 | 0.3 | 0.2 | 0.2 | - | - | 0.3 |
| Sodium perborate | 1.0 | - | - | - | - | - | - |
| Sodium Hypochlorite | - | - | - | 1.0 | 1.0 | 1.0 | 1.0 |
| Sodium percarbonate | - | - | - | - | - | - | - |
| Photobleach | - | - | 0.005 | - | - | - | - |
| Suds suppressors | 0.2 | 6.4 | - | - | 0.4 | 0.4 | 0.2 |
| Bleach catalyse | 1.0 | 0.5 | 0.5 | - | - | - | - |
| Water and minors⁴ | Balance | Balance | Balance | Balance | Balance | Balance | Balance |

| | | | | | | | |
|---|---|---|---|---|---|---|---|
| 1 Sulfonated/carboyxlated polymer "B" with 78 mole % AA, 25 mole % MA, 1 mole % SMS, 1% SPME and 0 mole % STY. 2 Hydrophobically modified, sulfonated/carboyxlated polymer "E" with 80.9 mole % AA, 0 mole % MA, 18 mole % STY, 0.62% SMS and 0.5 mole % SPME. 3 5,12-dimethyl-1,5,8,12-tetraaza-bicyclo[6.6.2]hexadecanemanganese (II) chloride. 4 Balance to 100% can, for example, include minors like bleach catalysts inter alia, 1,5-bis(hydroxymethylene)-3,7-dimethyl-2,4-bis(2-pyridyl)-3,7-diazabicyclo[3.3.1]-nonan-9-ol manganese(II) dichloride 1/2H2O, dispersants, inter alia, PEI 189 E15-18 according to U.S. Pat. No. 4,597,898 Vander Meer, issued Jul. 1, 1986, or PEI 1800 E7 according to U.S. Pat. No. 5,565,145 Watson et al., issued Oct. 15, 1996, optical brightener, perfume, suds suppresser, soil release agents, inter alia, according to U.S. Pat. No. 4,702,857 Gosselink, issued Oct. 27, 1987, or U.S. Pat. No. 4,968,451, Scheibel et al., issued Nov. 6, 1990, chelating agents, dye transfer inhibiting agents, additional water, and fillers, including CaCO3, talc, silicates, etc. | | | | | | | |

**TABLE VI**

| Heavy-Duty Liquid Laundry Detergent Composition | | | | | | |
|---|---|---|---|---|---|---|
| INGREDIENTS | EXAMPLES | | | | | |
| | 33 | 34 | 35 | 36 | 37 | 38 |
| C14-C15 alkyl E1.0 sulfate | 22.5 | 22.5 | 22.5 | 22.5 | - | - |
| Sodium C14-C15 alcohol sulfate | - | - | - | - | 4.5 | 11.2 |
| Sodium C14-C15 alcohol ethoxylate (6.5) | - | - | - | - | 0.5 | 1.0 |
| Linear alkyl benzene sulfonate | 3.0 | 3.0 | 3.0 | 3.0 | - | - |
| Sodium C11-C13 alkylbenzene sulfonate | - | - | - | - | 10.4 | 11.1 |
| C10 amidopropyl DMA | 1.5 | 1.5 | 1.5 | 1.5 | - | - |
| C12-C14 alkyl E7.0 | 3.0 | 3.0 | 3.0 | 3.0 | - | - |
| Citric Acid | 2.5 | 2.5 | 2.5 | 2.5 | - | - |
| C12-C18 alkyl fatty acid | 3.5 | 3.5 | 3.5 | 3.5 | - | - |
| Sodium carbonate | - | - | - | - | 25.2 | 16.1 |
| Sodium silicate (1:6 ratio NaO/ SiO2)(46%) | - | - | - | - | 2.1 | 2.6 |
| Sodium sulfate | - | - | - | - | 8.2 | 15.0 |
| Tallow fatty acid | - | - | - | - | - | 1.1 |
| Rapeseed fatty acid | 5.0 | 5.0 | 5.0 | 5.0 | | |
| Zeolite A, hydrate (0.1-10 micron size) | - | - | - | - | 21.3 | 28.0 |
| Protease | 0.8 | 1.57 | 1.57 | 1.57 | - | - |
| Amylase | 0.055 | 0.088 | 0.088 | 0.088 | - | - |
| Cellulase | 0.188 | 0.055 | 0.055 | 0.055 | - | - |
| Lipolase | 0.06 | - | - | - | - | - |
| mannanase | 0.007 | 0.0033 | 0.0033 | 0.0033 | - | - |
| Sodium metaborate | 2.0 | 2.5 | 2.5 | 2.5 | - | - |
| Ca formate/CaCl2 | 0.02 | 0.10 | 0.10 | 0.10 | - | - |
| Polyamine | 1.0 | 2.0 | 2.0 | 3.5 | - | - |
| Polymer¹ | 1.0 | 1.0 | 1.0 | 1.0 | 1.0 | 1.0 |
| Sodium perborate | - | - | - | - | 5.0 | - |
| Bleach activator² | - | - | - | - | 5.9 | - |
| Bleach catalyse | 0.035 | 0.034 | 0.034 | 0.034 | - | - |
| Hydrophobic dispersant⁴ | 0.65 | 0.76 | 0.76 | 0.76 | | |
| Poly(ethyleneglycol), MW ^{~}4000 (50%) | - | - | - | - | 1.0 | 1.1 |
| Soil release agent⁵ | - | - | - | - | 0.10 | 0.10 |
| Soil release agent⁶ | 0.147 | - | - | - | - | - |
| Soil release agent ⁷ | - | 0.10 | 0.10 | 0.10 | - | - |
| Suds suppresser | 0.60 | 0.60 | 0.60 | 0.60 | 0.60 | 0.60 |
| Water and minors⁸ | Balance | Balance | Balance | Balance | Balance | Balance |
| pH (1% Solution) | 9 | 9.8 | 10 | 10.5 | 10.5 | 11.5 |

| | | | | | | |
|---|---|---|---|---|---|---|
| 1 Hydrophobically modified, sulfonated/carboyxlated polymer "E" with 80.9 mole % AA, 0 mole % MA, 18 mole % STY, 0.62% SMS and 0.5 mole % SPME. 2 Nonyl ester of sodium p-hydroxybenzene-sulfonate. 3 1,5-bis(hydroxymethylene)-3,7-dimethyl-2,4-bis(2-pyridyl)-3,7-diazabicyclo[3.3.1]-nonan-9-ol manganese(II) dichloride 1/2H2O. 4 PEI 189 E15-18 according to U.S. Pat. No. 4,597,898 Vander Meer, issued Jul. 1, 1986. 5 Soil release agent according to U.S. Pat. No. 5,415,807 Gosselink et al., issued May 16, 1995 6 Soil release agent according to U.S. Pat. No. 4,702,857 Gosselink, issued Oct. 27, 1987. 7 Soil release agent according to U.S. Pat. No. 4,968,451, Scheibel et al., issued Nov. 6, 1990. 8 Balance to 100% can, for example, include minors like optical brightener, perfume, polymers, soil dispersant, chelating agents, dye transfer inhibiting agents, additional water, and fillers, including CaCO3, etc. | | | | | | |

**TABLE VII**

| Hard Surface Cleaning Composition | | | | | | | |
|---|---|---|---|---|---|---|---|
| INGREDIENTS | EXAMPLES | | | | | | |
| | 39 | 40 | 41 | 42 | 43 | 44 | 45 |
| Polymer¹ | 0.05 | - | - | 0.5 | - | - | 0.5 |
| Polymer² | - | 1.0 | - | - | 0.5 | - | 0.5 |
| Polymer³ | - | - | 0.10 | - | - | 1.0 | 1.0 |
| C9-11 alcohol ethoxylate (5.0) | - | 3.0 | - | - | - | - | - |
| C12-14 alcohol ethoxylate (5.0) | - | 2.0 | - | - | - | - | - |
| C12-14 alcohol ethoxylate (21) | - | - | 0.05 | - | - | - | - |
| C12-14 Cocamido propyl sulfobetaine | - | - | 0.22 | - | - | - | - |
| C12-14 Cocamidopropyl betaine | - | - | - | 0.20 | - | - | - |
| C10 Alkyl Polyglucoside | 0.05 | - | - | - | - | 10.0 | 10.0 |
| Sodium C10 Sulfate | - | - | - | - | 3.0 | - | - |
| Linear Alkyl Benzene Sulfonate | - | 0.25 | - | - | - | - | - |
| Ethanolamine | - | - | - | 0.50 | - | - | - |
| Sodium carbonate | | 0.5 | - | - | - | - | - |
| 2-amino-2-methyl-1- propanol | 0.01 | - | - | 0.5 | - | - | - |
| Propylene glycol n- butyl ether | 1.0 | - | 2.2 | 2.0 | - | - | - |
| Dipropylene glycol n-butyl ether | - | - | - | - | 4.0 | - | - |
| Ethanol | 3.0 | - | 8.0 | 3.0 | - | - | - |
| Didecyl dimethyl ammonium chloride | - | - | - | 0.3 | - | - | - |
| Xanthan Gum | - | - | - | - | 0.05 | - | - |
| Modified Polyethylene imines⁵ | 0.2 | - | - | - | - | - | - |
| Polyzwitterionic polymer⁶ | - | - | - | - | - | 3.0 | 3.0 |
| Poly(hexamethylene) biguanide | - | - | 0.30 | 0.10 | - | - | - |
| Citric Acid (50%) | - | - | 0.50 | - | 4.5 | - | - |
| Tartaric acid | - | - | - | 0.25 | - | - | - |
| NaOH (50%) | - | - | - | - | 0.6 | - | - |
| Water and minors⁷ | Balance | Balance | Balance | Balance | Balance | Balance | Balance |
| pH (10% Solution) | 9.0 | 10.5 | 3.0 | 11.0 | 3.0 | 5.0 | 5.0 |

| | | | | | | | |
|---|---|---|---|---|---|---|---|
| 1 Hydrophobically-modified, sulfonated/carboyxlated polymer "E" with 80.9mole % AA, 0mole % MA, 18mole % STY, 0.62% SMS and 0.5mole % SPME. 2 Sulfonated/carboyxlated polymer "B" with 78mole % AA, 25mole % MA, 1 mole % SMS, 1 % SPME and 0mole % STY. 3 Sulfonated/carboyxlated polymer "C" with 78mole % AA, 20mole % MA, 1mole % SMS, 1 % SPME and 0mole % STY. 4 A mixture of N-alkyl dimethyl ethylbenzyl ammonium chloride and N-dimethyl benzyl alkyl ammonium chloride may be provided. 5 Lupasol SK from BASF Corporation. 6 Mirapol HSC-300 from Rhodia Corporation. 7 Balance to 100% can, for example, include dyes, perfumes, speckles, corrosion inhibitor, hydrotropes, solvents, polymers, and additional water. | | | | | | | |

**TABLE VIII**

| Light-duty Liquid Detergent Composition | | | | | | | |
|---|---|---|---|---|---|---|---|
| INGREDIENTS | EXAMPLES | | | | | | |
| | 46 | 47 | 48 | 49 | 50 | 51 | 52 |
| Polymer¹ | 1.0 | 1.0 | 1.0 | - | - | - | - |
| Polymer² | - | - | - | - | 1.0 | - | 1.0 |
| Polymer³ | - | - | - | 1.0 | - | 1.0 | - |
| Poly (dimethylaminomethacrylate) Suds Boosting Polymer | 0.2 | - | - | 0.2 | 0.2 | 0.2 | 0.2 |
| Bis(aminomethyl) cyclohexane diamine | 0.5 | 0.5 | 0.5 | 0.5 | 0.5 | 0.5 | 0.5 |
| Alkyl Ethoxy (0.6) Sulfate | 26.5 | 26.5 | 26.5 | 26.5 | 26.5 | 26.5 | 26.5 |
| C9E11 Nonionic (Neodol 9-11) | 3.0 | 3.0 | 3.0 | 3.0 | 3.0 | 3.0 | 3.0 |
| C12 Dimethyl Amine Oxide | 6.0 | 6.0 | 6.0 | 6.0 | 6.0 | 6.0 | 6.0 |
| Ethanol | 4.0 | 4.0 | 4.0 | 4.0 | 4.0 | 4.0 | 4.0 |
| Sodium Cumene Sulfonate | 4.0 | 4.0 | 4.5 | 4.0 | - | 4.0 | - |
| Amylase Enzyme | 0.2 | 0.2 | - | 0.2 | - | 0.2 | - |
| Protease Enzyme | 0.5 | 0.5 | - | 0.5 | 0.5 | - | 0.5 |
| Water and minors ⁴ | Balance | Balance | Balance | Balance | Balance | Balance | Balance |
| pH (10% Solution) | 9.0 | 9.0 | 9.0 | 9.0 | 9.0 | 9.0 | 9.0 |

| | | | | | | | |
|---|---|---|---|---|---|---|---|
| 1 Hydrophobically modified, sulfonated/carboyxlated polymer "E" with 80.9 mole % AA, 0 mole % MA, 18 mole % STY, 0.62% SMS and 0.5 mole % SPME. 2 Sulfonated/carboyxlated polymer "B" with 78 mole % AA, 25 mole % MA, 1 mole % SMS, 1% SPME and 0 mole % STY. 3 Sulfonated/carboyxlated polymer "C" with 78 mole % AA, 20 mole % MA, 1 mole % SMS, 1% SPME and 0 mole % STY. 4 Balance to 100% can, for example, include dyes, perfumes, speckles, corrosion inhibitor, and additional water. | | | | | | | |

**TABLE IX**

| Chemical Composition of the Sulfonated/carboxylated Polymers | | | | | | | |
|---|---|---|---|---|---|---|---|
| Polymer | MW | MONOMERS (% MOLE) | | | | | |
| | | AA | MMA | STY | SMS | SPME | MAA |
| Polyacrylate¹ | <10 | 100 | 0 | 0 | 0 | 0 | 0 |
| A | 20.5 | 68 | 30 | 0 | 1 | 1 | 0 |
| B | 20.4 | 73 | 25 | 0 | 1 | 1 | 0 |
| C | 20.3 | 78 | 20 | 0 | 1 | 1 | 0 |
| D | 27.3 | 80 | 0 | 18 | 1 | 1 | 0 |
| E | 49.1 | 80.88 | 0 | 18 | 0.62 | 0.5 | 0 |
| F | 20.2 | 89 | 0 | 10 | 0.57 | 0.45 | 0 |
| G | 13.7 | 94 | 0 | 5 | 0.57 | 0.45 | 0 |

| | | | | | | | |
|---|---|---|---|---|---|---|---|
| 1 A unmodified polyacrylate having a molecular weight less than about 10 kDa. | | | | | | | |

**TABLE X**

| Key To Acronyms | |
|---|---|
| MW | Weight average molecular weight. |
| AA | Acrylic acid |
| AMPS | 2-acrylamido-2methyl-propansulphonic |
| SMS | Sodium methallyl sulfonate |
| MAA | Methacrylic acid |
| MMA | Methyl methyacrylate |
| SPME | Sulfophenylmethallylether |
| STY | Styrene |

It should be understood that every maximum numerical limitation given throughout this specification would include every lower numerical limitation, as if such lower numerical limitations were expressly written herein. Every minimum numerical limitation given throughout this specification will include every higher numerical limitation, as if such higher numerical limitations were expressly written herein. Every numerical range given throughout this specification will include every narrower numerical range that falls within such broader numerical range, as if such narrower numerical ranges were all expressly written herein.

## Claims

1. A surfac-treating composition, comprising:
a) an effective amount of a water-soluble, sulfonated/carboxylated polymer having a molar content, said polymer comprising:
(i) at least one carboxylic acid functionality;
(ii) optionally, one or more nonionic functionality; and
(iii) at least one sulfonate functionality, wherein said sulfonate functionality is less than or equal to 2 mole % of the molar content of said polymer; and
b) at least one adjunct ingredient.

2. The surface-treating composition according to Claim 1 wherein said at least one carboxylic acid functionality comprises at least one structural unit derived from at least one carboxylic monomer having the general formula (I): wherein R1 to R4 are independently hydrogen, methyl, carboxylic acid group or CH2COOH and wherein said carboxylic acid groups can be neutralized.

3. The surface-treating composition according to Claim 1 wherein said one or more nonionic functionality comprises at least one structural unit derived from at least one nonionic monomer having the general formula (II): wherein R⁵ is hydrogen, C₁ to C₆ alkyl or C₁ to C₆ hydroxyalkyl, and X is either aromatic (with R⁵ being hydrogen or methyl when X is aromatic) or X is of the general formula (III): wherein R⁶ is (independently of R⁵) hydrogen, C₁ to C₆ alkyl, or C₁ to C₆ hydroxyalkyl, and Y is O or N.

4. The surface-treating composition according to Claim 1 wherein said at least one sulfonate functionality comprises at least one structural unit derived from at least one sulfonate monomer having the general formula (IV): wherein R⁷ is a group comprising at least one sp² bond, A is O, N, P, S or an amido or ester linkage, B is a mono- or polycyclic aromatic group or an aliphatic group, each is independently 0 or 1, and M⁺ is a cation. In one aspect, R⁷ is a C₂ to C₆ alkene. In another aspect, R⁷ is ethane, butene or propene.

5. The surface-treating composition according to Claim 4 wherein R⁷ is selected from the group consisting of a C₂ to C₆ alkene, ethane, butene, propene, and combinations thereof.

6. The surface-treating composition according to Claim 1 wherein said polymer has a weight-average molecular weight of less than or equal to about 100,000 Da.

7. The surface-treating composition according to Claim 1 wherein said polymer comprises: (a) from 0.01 mole % to 2 mole % of a sulfonate functionality; and (b) less than or equal to 99,99 mole % of a carboxylic acid functionality.

8. The surface-treating composition according to Claim 7 wherein said sulfonate functionality comprises one or more of the following: sodium (meth) allyl sulfonate, vinyl sulfonate, sodium phenyl (meth) allyl ether sulfonate, 2-acrylamido-methyl propane sulfonic acid, and combinations hereof.

9. The surface-treating composition according to Claim 7 wherein said at least one carboxylic acid functionality is selected from the group consisting of acrylic acid, maleic acid, itaconic acid, methacrylic acid, ethoxylate esters of acrylic acids, and combinations thereof

10. The surface-treating composition according to Claim 1 wherein said polymer comprises (a) from 99.98% to 48% of a carboxylic acid functionality, (b) from 0.01% to 50% of a nonionic functionality; and (c) from 0.01% to less than or equal to 2% of a sulfonate functionality.

11. The surface-treating composition according to Claim 1 wherein said at least one nonionic functionality is selected from the group consisting of methyl (meth) acrylate, ethyl (meth) acrylate, t-butyl (meth) acrylate, methyl (meth) acrylamide, ethyl (meth) acrylamide, t-butyl (meth) acrylamide, styrene, α-methyl styrene, and combinations thereof

12. The surface-treating composition according to Claim 11 wherein said nonionic functionality contains an aromatic moiety.

13. The surface-treating composition according to Claim 12 wherein said aromatic moiety is styrene.

14. The surface-treating composition according to Claim 1 wherein said polymer does not contain an ester and/or amide functionality.

15. The surface-treating composition according to Claim 1 wherein said surface-treating composition is provided in one of the following forms: solid, granule, powder, liquid, paste, cream, gel, or liquigel.

16. The surface-treating composition according to Claim 15 wherein said surface-treating composition is provided in a unitized dose in one of the following forms: tablet, gel pack, capsule, multi-compartment capsule, water-soluble pouch, or multi-compartment pouch.

17. The surface-treating composition according to Claim 1 wherein said at least one adjunct ingredient comprises one or more of the following: aesthetic agents, anti-filming agents, antiredopsition agents; anti-spotting agents, beads, binders, bleach activators, bleach catalysts, bleach stabilizing systems, bleaching agents, brighteners, buffering agents, builders, carriers, chelants, color speckles, control release agents, corrosion inhibitors, clays, dishcare agents, disinfectant, dispersant agents, dispersant polymers, draining promoting agents, drying agents, dyes, dye release inhibiting agents, enzymes, enzyme stabilizing systems, fillers, free radical inhibitors, fungicides, germicides, hydrotropes, opacifiers, perfumes, pH adjusting agents, pigments, processing aids, silicates, soil release agents, suds suppressors, surfactants, stabilizers, and thickeners.

18. The surface-treating composition according to Claim 17 wherein said at least one adjunct ingredient comprises chlorine bleach.

## Patentansprüche

1. Oberflächenbehandlungs-Zusammensetzung, umfassend:
a) eine wirksame Menge eines wasserlöslichem, sulfonierten/carboxylierten Polymers mit Molgehalt, wobei Tdas polymer Folgendes umfasst:
(i) mindestens eine Carbonsäure-Funktionalität;
(ii) wahlweise eine oder mehrere nichtionische Funktionalitäten und
(iii) mindestens eine Sulfonat-Funktionalität, wobei die Sulfonat-Funktionalität weniger als oder gleich 2 Mol-% des Molgehalts des Polymers beträgt; und
b) zu übrigen Teilen Zusatzbestandteile.

2. Oberflächenbehandlungs-Zusammensetzung nach Anspruch 1, wobei die mindestens eine Carbonsäure-Funktionalität mindestens eine Struktureinheit umfasst, die von mindestens einem Carboxylmonomer mit der folgenden allgemeinen Formel (I) abgeleitet ist: worin R1 bis R4 jeweils unabhängig voneinander eine Wasserstoff-, Methyl- oder Carbonsäuregruppe oder CH2COOH sind und worin die Carbonsäuregruppen neutralisiert sein können.

3. Oberflächenbehandlung-Zusammensetzung nach Anspruch 1, wobei die eine oder die mehreren nichtionischen Funktionalitäten mindestens eine Struktureinheit umfassen, die von mindestens einem, nichtionischen Monomer der folgenden allgemeinen Formel (II) abgeleitet sind: worin R⁵ Wasserstoff, C₁- bis C₆-Alkyl oder C₁- bis C₆-Hydroxyalkyl ist und X entweder aromatisch ist (wobei R⁵ Wasserstoff oder Methyl ist, wenn X aromatisch ist) oder X die folgende allgemeine Formel (III) hat: worm R⁶ (unabhängig von R⁵) Wasserstoff, C₁- bis C₆-Alkyl oder C₁- bis (C₆-Hydroxyalkyl ist und Y für O oder N steht.

4. Oberflächenbehandlungs-Zusammensetzung nach Ansprach 1, wobei die mindestens eine Sulfonat-Funktionalität mindestens eine Struktureinheit umfasst, die von mindestens einem Sulfonatmonomer mit der folgenden allgemeinen Formel (IV) abgeleitet ist: worin R⁷ eine Gruppe ist, die mindestens eine sp²-Bindung umfasst, A für O, N, P, S oder eine Amido- oder Esterbindung steht, B eine mono- oder polycyclische aromatische Gruppe oder eine aliphatische Gruppe ist, jedes unabhängig 0 oder 1 ist und M⁺ ein Kation ist. In einem Aspekt ist R⁷ ein C₂- bis C₆-Alken. In einem anderen Aspekt ist R⁷ Ethan, Buten oder Propen.

5. Oberflächenbehandlungs-Zusammensetzung nach Anspruch 4, wobei R⁷ ausgewählt ist aus der Gruppe, bestehend aus einem C₂- bis C₆-Alken, -Ethan, -Buten, -Propen und Kombinationen davon.

6. Oberflächenbehandlungszusammensetzung nach Anspruch 1, wobei das Polymer ein vor, weniger als oder ungefähr gleich 100.000 Da hat.

7. Oberflächenbehandlungs-Zusammensetzung nach Anspruch 1, wobei das Polymer Folgendes umfasst: (a) zu 0,01 Mol-% bis 2 Mol-% eine Sulfonat-Funktionalität; und (b) zu weniger als oder zu 99,99 Mol-% eine Carbonsäure-Funktionalität.

8. Oberflächenbehandlungs-Zusammensetzung nach Anspruch 7, wobei die Sulfonat-Funktionalität eines oder mehrere der Folgenden umfasst: Natrium-(meth)allylsulfonat, Vinylsulfonat, Natriumphenyl(meth)allylethersulfonat, 2-Acrylamidomethylpropansulfonsäure und Kombinationen davon.

9. Oberflächenbehandlungs-Zusammensetzung nach Anspruch 7, wobei, die mindestens eine Carbonsäure-Funktionalität ausgewählt ist aus der Gruppe, bestehend aus Acrylsäure. Maleinsäure, Itaconsäure, Methacrylsäure, Ethoxylatestern von Acrylsäuren und Kombinationen davon.

10. Oberflächenbehandlungs-Zusammensetzung nach Anspruch 1, wobei das Polymer (a) zu 99,98 % bis 48 % eine Carbonsaure-Funktionalität, (b) zu 0,01 % bis 50 % eine nichtionische Funktionalität; und (c) zu 0,01 % bis höchstens 2 % eine Sulfonat-Funktionalität umfasst.

11. Oberflächenbehandlungs-Zusammensetzung nach Anspruch 1, wobei die mindestens eine nichtionische Funktionalität ausgewählt ist aus der Gruppe, bestehend aus Methyl(meth)acrylat, Ethyl(meth)acrylat, t-Butyl(meth)acrylat, Methyl(meth)acrylamid, Ethyl(meth)acrylamid, t-Botyl(meth)acrylamid, Styrol, α-Methylstyrol und Kombinationen davon.

12. Obernächenbehandlungs-Zusamnensetzung nach Anspruch 11, wobei die nichtionische Funktionalität eine aromatische Einheit enthält.

13. Oberflächenbehandinngs-Zusammeasetzung nach Anspruch 1 2, wobei die aromatische Einheit Styrol ist.

14. Oberflächenbehandlungs-Zusammensetzung nach Anspruch 1, wobei das Polymer kerne Ester- und/ode Amid-Funktionalität enthält.

15. Oberflächenbehandlungs-Zusammensetzung nach Anspruch 1, wobei die Oberflächenbehandlungs-Zusammensetzung in einer der folgenden Formen bereitgestellt wird: Feststoff, Granulat, Pulver, Flüssigkeit, Paste, Creme, Gel oder RüssiggeL

16. Oberflächenbehandlunngs-Zusammensetzung nach Anspruch 15, wobei die. Oberflächenbehandlungs-Zusammensetzung in einer Einheilsdosis in einer der folgenden Formen bereitgestellt wird: Tablette, Gelpackung, Kapsel. Mehrkammerkapsel, wasserlöslicher Beutel oder Mehrkammerbeutel.

17. Oberflächenbehandinsgs-Zusammensetzung nach Anspruch 1 , wobei der mindestens eine Zusatzbestandteil eines oder mehrere der Folgenden umfasst:
ästhetische Mittel, Mittel gegen Filmbildung, Antiwiederablagerungsmittel, Mittel gegen Fleckenbildung, Kügelchen, Bindemittel, Bleichaktivatoren, Bleichmittelkatalysatoren, Bleichmittel-Stabilisierungssysteme, Bleichmittel, Aufheller, Puffermittel, Builder, Träger, Komplexbildner, Farbsprenkel, Freisetzungssteuerungsmittel, Korrosionsschutzmittel, Tonerden, Geschirrpflegemittel, Desinfektionsmittel, Dispergiermittel, dispergierende Polymere, ablauffördernde Mittel, Trockenmittel, Farbstoffe, Farbstoffabgabehemmer, Enzyme, Enzymstabilisierungssysteme, Füllmittel, Radikalhemmer, pilztötende Mittel, keimtötende Mittel, Hydrotropika, Trübungsmittel, Duftstoffe, pH-Regler, Pigmente, Verarbeitungshilfsmittel, Silicate, Schmutzabweisemittel, Schaumunterdrücker, Tenside, Stabilisierungsmittel und Verdickungsmittel.

18. Oberflächenbehandlungs-Zusammensetzung nach Anspruch 17, wobei der mindestens eine Zusatzbestandteil Chlorbleichmittel umfasst.

## Revendications

1. Composition de traitement de surface, comprenant :
a) une quantité efficace d'un polymère sulfoné/carboxylate hydrosoluble ayant une teneur molaire, ledit polymère comprenant ;
(i) au moins une fonctionnalité acide carboxylique ;
(ii) facultativement, une ou plusieurs fonctionnalités non ionique ; et
(iii) au moins une fonctionnalité sulfonate, où ladite fonctionnalité sulfonate est inférieure ou égale a 2% molaires de la teneur molaire dudit et
b) au moins un ingrédient additif.

2. Composition de traitement de surface selon la revendication 1, dans laquelle ladite au moins une fonctionnalité acide carboxylique comprend au moins un motif structural dérivé d'au moins un monomère carboxylique de de formule générale (I) : dans laquelle R1 à R4 sont indépendamment un hydrogène, un méthyle, un groupe acide carboxylique ou CH2COOH et dans laquelle lesdits groupes acide carboxylique peuvent être neutralisés.

3. Composition de traitement de surface selon la revendication 1, dans laquelle ladite une ou plusieurs fonctionnalités non ioniques comprennent au moins un motif structural dérive d'au moins un monomère non ionique, de formule générale (II) : dans laquelle R⁵ est un hydrogène, un alkyle en C₁ à C₆, ou un hydroxyalkyle en C₁ à C₆, et X est ou aromatique (avec R⁵ étant un hydrogène ou un méthyle lorsque X est aromatique) ou est de formule générale (III) : dans laquelle R⁶ est (indépendamment de R⁵) un hydrogène, un alkyle en C₁ à C₆, ou un hydroxyalkyle en C₁ à C₆, et Y est O ou N.

4. Composition de traitement de surface selon la revendication 1, dans laquelle ladite au moins une fonctionnalité sulfonate comprend au moins un motif structural dérive d'au moins un monomère sulfonate de formule générale (IV) : dans laquelle R⁷ est un groupe comprenant au moins une liaison sp², A est Q, N, P, S ou une liaison amido ou ester, est un groupe aromatique mono- ou polycyclique ou un groupe aliphatique, chaque t est indépendamment 0 ou 1, et M⁺ est un cation. Sous un aspect, R⁷ est un alcène en C₂ à C₆ Sous un autre aspect, R⁷ est un éthane, un butène ou un propène;

5. Composition de traitement de surface selon a revendication 4, dans laquelle R⁷ est choisi dans le groupe constitue en C₂ à C₆, éthane, butène, propène, et leurs combinaison.

6. Composition de traitement de surface selon la revendication 1, dans laquelle ledit polymère a une masse moléculaire moyenne en poids inférieure ou égale à environ 100 000 Da.

7. Composition de traitement de surface selon la revendication 1, dans laquelle ledit polymère comprend ; (a) de 0,01 % molaire à 2 % molaires d'une fonctionnalité sulfonate ; et (b) une teneur inférieure ou égale à 99,99 % molaires d'une fonctionnalité acide carboxylique.

8. Composition de traitement de surface selon la revendication 7, dans laquelle ladite fonctionnalité sulfonate comprend une ou plusieurs des substances suivantes : sodium (méth) allyl sulfonate, vinyl sulfonate, sodium phényl (méth) allyl éther sulfonate, acide 2-acrylamido-méthylpropane sulfonique, et leurs combinaisons.

9. Composition de traitement de surface selon la revendication 7, dans laquelle ladite au moins une fonctionnalité acide est choisie dans le groupe constitue d'acide acrylique, acide maléique, acide itaconique, acide méthacrylique, esters d'éthoxylate d'acides acryliques, et leurs combinaisons.

10. Composition, de traitement de surface selon In revendication 1, dans laquelle ledit polymère comprend (a) de 99,98 % à 48 % d'une fonctionnalité acide carbonique, (b) de 0,01 % à 50 % d'une fonctionnalité non ionique ; et de 0,01 % jusqu'à une teneur inférieure ou égale à 2 % d'une fonctionnalité sulfonate.

11. Composition de traitement de surface selon la revendication 1, dans laquelle ladite au moins une fonctionnalité non ionique est choisie dans le groupe constitue de méthyl (méth) acrylate, éthyl (méth) acrylate, t-butyl (méth) acrylate, méthyl (méth) acrylamide, éthyl(méth) acrylamide, t-butyl (méth) acrylamide, styrène, α-methyl styrène, et leurs combinaisons.

12. Composition de traitement de surface selon la revendication 11, dans laquelle ladite fonctionnalité non ionique contient un fragment aromatique.

13. Composition de traitement de surface selon la revendication 12, dans laquelle ledit fragment aromatique est du styrène,

14. Composition de traitement de surface selon la revendication 1, dans laquelle ledit polymère ne contient pas de fonctionnalité ester et/ou amide.

15. Composition de traitement de surface selon la revendication 1, où ladite composition de traitement de surface est fournie sous une des formes suivantes : solide, granule, poudre, liquide, pâte, crème, gel ou liquigel.

16. Composition de traitement de surface selon lit revendication 15, où ladite composition de traitement, de surface est fournie dans une dose unitaire sous une des formes suivantes : tablette, gel pack, capsule, capsule à compartiments multiples, sachet hydrosoluble, ou sachet à compartiments multiples.

17. Composition de traitement de surface selon la revendication 1, dans laquelle ledit au moins un ingrédient additif comprend une ou plusieurs des substances suivantes : agents esthétiques, agents anti-filmogènes, agents antiredéposition, agents antitaches, pertes, liants, activateurs de blanchiment, catalyseurs de blanchiment, système de stabilisation d'agent de blanchiment, agents de blanchiment, azurants agents tampons, adjuvants, véhicules, agents chélatants, particules de couleur, agents de contrôle de libération, inhibiteurs de corrosion, argiles, agents de soin de la vaisselle, désinfectant, agents dispersants, polymères dispersants, agents favorisant le drainage, agents desséchants, teintures, agents inhibiteurs de décoloration, enzymes, systèmes de stabilisation des enzymes, charges, inhibiteurs de radicaux libres, fongicides, germicides, hydrotropes, opacifiants, parfums, agents d'ajustement du pH, pigments, auxiliaires de traitement, silicates, agents de libération des salissures, suppresseurs de mousse, agents tensioactifs, agents stabilisants, et épaississants.

18. Composition de traitement de surface, selon la revendication 17, dans laquelle ledit au moins un ingrédient additif comprend un agent de blanchiment au chlore.
